

Patented Mar. 2, 1926.

1,575,052

## UNITED STATES PATENT OFFICE.

LEOPOLD HESSE, OF BARMEN, AND HERMANN RATHERT, OF ELBERFELD, GERMANY.

PROCESS OF MANUFACTURING THIN THREADS OF ARTIFICIAL SILK OF HIGHEST DEGREE OF FINENESS FROM VISCOSE.

No Drawing.

Application filed February 13, 1922. Serial No. 536,365.

To all whom it may concern:

Be it known that we, LEOPOLD HESSE, a citizen of the German Empire, residing at Barmen, Germany, and HERMANN RATHERT, a citizen of the German Empire, residing at Elberfeld, Germany, have invented certain new and useful Processes of Manufacturing Thin Threads of Artificial Silk of Highest Degrees of Fineness from Viscose (for which we have filed applications in Germany February 28th, 1921; Holland, September 1st, 1921), of which the following is a specification.

Thin threads of artificial silk from viscose of very high degrees of fineness could only be obtained heretofore from viscose solutions as heretofore known by keeping within the limits of sharply defined conditions of maturing of such solutions which should have very exact sharply defined compositions with a view of obtaining certain individual thread numbers or titers. Thus for instance, by the ejection of viscose solutions from nozzles with apertures of one-tenth millimeter diameter, and by employing a velocity of the reeling mechanism up to fifty meters per minute.

1/and by using acid spinning baths with an excess of neutral sulfate over the bisulfate present threads were obtained having individual numbers down to four deniers; while

2/in strongly acid precipitating baths with an excess of free sulphuric acid over the bisulphate highly glossy threads were obtained of a size numbering down to 2 deniers;

3/baths of sulfate of ammonia mixed with but little acid yield extremely fine threads of viscose artificial silk having individual thread numbers below 2 deniers.

Now, as distinguished from this previous state of the art our invention relates to a process according to which, aside from threads above five deniers, highly glossy very thin artificial silk threads below .5 deniers, as well as glossy threads of artificial silk of high degrees of fineness below two deniers may be obtained by employing the same spinning bath and the same viscose of the same degree of maturity, and with nozzles having apertures of the same diameter.

Our process substantially resides in the precipitation of certain solutions of viscose

by means of a spinning bath containing sulfate of soda, and showing a degree of acidity of about 15 to 16 percent of sulphuric acid at a specific gravity of about 1.39 to 1.45 at 40 degrees centigrade, the precipitation being effected at temperatures ranging from 35 to 50 degrees centigrade. And the invention is particularly distinguished by the fact that both the treatment with carbon-bisulphide as well as the dissolving of the xanthate obtained thereby are effected in the presence of reducing agents of which we prefer the use of alkali sulphite. With a view of simplifying the process and of economizing reducing agent we may proceed by using the waste liquor obtained by the separation of the alkali-cellulose from the liquid previous to the action of carbon-bisulphide as a solvent for the xanthate produced. In a general way such solutions of viscose are obtained by first preparing the xanthogenate of cellulose by the treatment with carbon-bisulfide of alkali-cellulose at the exclusion of the action of oxygen from the air, and preferably with the addition of reducing agents, and then dissolving such xanthogenate in pure or previously used liquors containing reducing agents, these solutions being then precipitated as hereinbefore referred to. The products obtained may be converted into threads by using nozzles with apertures of one tenth millimeter diameter, and having withdrawing velocities for the escaping threads up to .50 meters.

The maturity and the age of the viscose to be submitted to the spinning operation with this invention are capable of variation within unsurpassedly wide limits, so that by this new process a very important improvement over the present state of the art is realized. While, with the ordinary kinds of viscose and by using the usual acid precipitating baths, the duration of maturity for the viscose should not vary for more than about twelve hours at the ordinary temperature, without jeopardizing the quality of the spun material and of the threads themselves, it has become possible in accordance with this invention, to submit the viscose to the spinning operation within a multiple of the period referred to and within a period of maturity of 13, 2 to 6, glossy thin threads of very high degrees of fineness being obtained in this manner. An

additional advantage is realized by the new process by the fact that it becomes possible to avoid the very annoying generation of sulfide of hydrogen during the spinning operation by correspondingly adjusting the addition of sulfite, inasmuch as the gaseous sulfuretted hydrogen and sulphurous acid developing at the moment of coagulation are decomposed with the formation of sulfur.

The composition of the precipitating bath may be varied within certain limits, so that it is possible to use baths of an acidity which is above or below the contents above referred to for several percentages.

With equally favorable results the new process may be applied for the manufacture of staple fibers up to the very finest single threads.

In the practice of our invention we may, for instance, proceed as follows:—

*Example I.*—2 kilograms of bleached sulfite pulp are mercerized at ordinary temperature for about ninety minutes in about 25 liters of soda liquor of 18 percent in which 315 grams crystallized sodium sulphite have been dissolved; the disintegrated comminuted alkali-cellulose is submitted to a preliminary maturing in closed boxes at 30 22 degrees centigrade for about 80 hours after having been squeezed out to about 6.2 kilograms. Then the alkali-cellulose is treated with about 600 grams of carbon-bisulfide at about 20 degrees cent. for 35 some hours with gentle agitation, and the xanthate formed is dissolved into viscose by treatment with 2½ kilograms soda lye of 18%, and 10½ kilograms of water at about 15 degrees C.

40 After repeated filtration the viscose is determined at a maturing stage between 13 and 7 by coagulation with ammonium-chloride solution according to Hottenroth this determination being effected by titrating, say twenty grams of viscose with a 10 percent solution of ammonium-chloride until coagulation occurs, as described in *Chemiker-Zeitung*, Cöthen, 1915, page 119; it is then injected in the quantity required for obtaining a titer or thread number of 125 deniers from a spinning nozzle having 30 holes of one-tenth millimeter diameter, and into a spinning bath of 42 degrees centigrade containing sodium-sulphate, and 55 having an acidity of from 15 to 16 percent sulphuric acid determined at 40 degrees C. and at a specific gravity of 1.459. The bundle of fibers obtained in this manner is wound upon a reel or bobbin in the usual manner, having a pulling velocity of 40 meters. The finished bobbin with the threads wound thereon is freed from acid and salt by washing it with water; it is then dried, twisted if desired, and submitted to 60 further treatment as usual. The thread of

artificial viscose silk is glossy after desulfuration. The single thread number or titer is about 4 deniers.

*Example II.*—The xanthate of cellulose obtained as described in the first example is dissolved at about 15 degrees centigrade with 9½ kilograms of water in 3.7 kilograms of waste alkali liquor of 16.4 percent obtained upon the mercerization or squeezing out of the alkali-cellulose, and containing soluble organic bodies and sulfite of sodium from the cellulose. The repeatedly filtered viscose in the quantity required for obtaining a titer-thread number of 60 deniers is injected from a nozzle with 40 holes of one tenth millimeter diameter each, and at an ammonium-chloride maturity stage of between 13 and 6, into a spinning bath of 42 degrees centigrade temperature which shows a density of 1.39 observed at 40 degrees C. The bath contains from 15 to 16 percent of sulphuric acid and enough sodium-sulphate to bring the specific gravity up to the required value. The thread obtained is treated as described with reference to Example I. The desulfurated thread is glossy, and possesses an individual single thread number or titer of 1.5 deniers.

Certain differences in the contents of cellulose, alkali and carbon-bisulfid, and certain variations of temperature are permissible without interference with the process. The amount of sulfite added to the viscose according to the procedure above described may be further increased by separate additions at any suitable points of the process.

We claim:—

1. The process of producing artificial silk threads from viscose, which consists in treating alkali-cellulose with carbon-bisulfide in the presence of a reducing agent, dissolving the xanthogenate formed in alkali in the presence of reducing agents, and injecting the solution obtained into a solution of sodium sulphate containing comparatively large amounts of sulphuric acid.

2. The process of producing artificial silk threads from viscose, which consists in treating alkali-cellulose with carbon-bisulfide in the presence of reducing agents, dissolving the xanthate produced in a mixture of alkaline liquor with sodium sulphite, ripening the solution, and then injecting the same into an acid setting and coagulating bath.

3. The process of producing artificial silk threads from viscose, which consists in treating alkali cellulose with carbon bisulfide in the presence of reducing agents, dissolving the xanthate formed in soda liquor containing sulphite of alkali, and injecting the solution obtained into a strongly acid solution of sodium sulphate.

4. The process of producing objects from viscose, which consists in treating cellulose

- with alkali in the presence of reducing agents, separating the alkali-cellulose obtained from the waste liquor, treating the alkali-cellulose with carbon-bisulphide, dissolving the xanthate thereby produced in said waste liquor, and introducing said solution into a setting and coagulating bath.
5. The process of producing objects from viscose, which consists in treating cellulose with alkali and sodium sulphite, submitting the alkali-cellulose obtained to a preliminary maturing, separating the alkali-cellulose from the waste liquor, treating the alkali-cellulose with carbon-bisulphide, dissolving 10 the xanthate thereby produced in said waste liquor, ripening the solution obtained and introducing the solution into a setting and coagulating bath.
6. The process of producing objects from 20 viscose, which consists in treating cellulose with alkali and sodium-sulphite, separating it from the waste liquor, submitting the alkali-cellulose obtained to a preliminary maturing, treating the alkali-cellulose with 25 carbon-bisulphide, dissolving it in alkali-solution containing sulphite of alkali, ripening the solution of viscose obtained, and introducing it at an ammonium-chloride measure of between 13 and 6 ripening stage 30 into a setting and coagulating bath.
7. The process of producing artificial silk from viscose, which consists in treating alkali-cellulose with carbon-bisulphide in

the presence of a reducing agent, dissolving the xanthogenate formed in alkali in the 35 presence of reducing agents, and treating the solution obtained with a setting bath.

8. The process of producing artificial silk material from viscose, which consists in treating alkali-cellulose with carbon-bisulphide and soluble sulphite, dissolving the xanthogenate formed in alkali in the presence of sulphite, and treating the solution obtained with a setting bath.

9. The process of preparing artificial-silk- 45 material from viscose, which consists in treating cellulose with caustic-alkali-liquor in the presence of soluble sulphite, removing the bulk of the liquid, and treating the remaining mass, containing sulphite with 50 carbon-bisulphide, and finally acting there-upon with a setting bath.

10. The process of preparing artificial-silk-material from viscose, which consists in treating cellulose with caustic-alkali-liquor 55 in the presence of soluble alkali-sulphite, removing the bulk of the liquid, treating the remaining mass in the presence of soluble sulphites with carbon-bisulphide, dissolving the xanthogenate formed in alkali in the 60 presence of reducing agents, and treating the solution obtained with a setting bath.

In testimony whereof we affix our signatures.

DR. L. HESSE.  
DR. H. RATHERT.